

## UNITED STATES PATENT OFFICE

2,635,078

## GREASE COMPOSITIONS

Fred H. Stross and Stanley T. Abrams, Berkeley,  
Calif., assignors to Shell Development Com-  
pany, Emeryville, Calif., a corporation of Dela-  
ware

No Drawing. Application November 27, 1950,  
Serial No. 197,836

7 Claims. (Cl. 252—25)

1

This invention relates to novel lubricant compositions. More particularly, it is concerned with lubricating compositions comprising lubricating proportions of an oleaginous liquid and an added agent possessing a combination of gelling and extreme pressure properties. The compositions are characterized by their ability to withstand high temperatures, excellent resistance to disintegration by water, and anti-friction properties at extreme pressures.

There have been disclosed to the art a number of fluid and grease-like compositions containing sulfurized materials especially for use as extreme pressure lubricants. In most instances, these compositions have contained either sulfurized fatty acids or sulfurized fatty oils. Where greases are desired particularly for use at high temperatures, such sulfurized materials show the shortcomings that the compositions are excessively corrosive and tend to soften or lose their grease-like structures progressively with increasing temperatures.

It has been proposed to add finely divided disulfides to silicone fluids, said disulfides being derived from metalloids such as molybdenum, tungsten and titanium. Such compositions may be useful under certain conditions of operation, but in many instances are unsatisfactory due to the unstable nature of the suspension. This unstable character appears to be due to two principal causes. In the first place, the disulfides previously used for this purpose, although called "colloidally fine," are not actually believed to be of such highly dispersed nature as to enable them to exist as a true colloidal gel. This is indicated from the fact that the disulfides are derived from ores which have been finely ground to an average dimension of 1 to 50 microns. Although these ground ores are subsequently subjected to various extraction treatments, it is not believed that this particle size is appreciably altered. On the other hand, true colloidal gel particles are defined as those having dimensions of between 0.001 and 0.1 micron. Secondly, according to the teachings of the art, these disulfides are of a plate-like structure in which it is postulated that three layers exist, namely, a middle metalloid layer having on either side a layer of sulfur atoms. Structures of this character exhibit little attraction between the molecular layers, and, hence, a true gel structure is not formed when the particles are dispersed in a liquid.

It is an object of the present invention to provide lubricating compositions exhibiting im-

2

proved extreme pressure characteristics. It is another object of the present invention to provide stable grease-like compositions especially effective as extreme pressure lubricants at elevated temperatures. It is a further object of the invention to provide compositions having the foregoing characteristics and in addition thereto being comparatively stable to the disintegrating influences of water. The foregoing and other objects will be understood from the following description of the invention.

Now in accordance with the present invention, it has been found that hydrocarbon lubricating oils are provided with grease-like structures by 15 the dispersal therethrough of colloidal gels of sulfides of metals having a water solubility no greater than 0.0005 g. per 100 cc. H<sub>2</sub>O at 20° C. Still in accordance with the present invention, it has been found that outstanding members of 20 the present series of greases comprise those gelled with copper sulfides, since copper sulfides exhibit peculiar oleophilic properties common to sulfides of the "hydrogen sulfide group" metals as compared with other metallic sulfide com- 25 pounds.

These colloidal particles have sizes varying from 0.01 to 0.3 micron, and usually between 0.01 and 0.1 micron. Electron micrographs indicate that the particles are three dimensional units 30 showing an agglomerating tendency which accounts for their stable gel-forming property. It has been found that, dependent in part upon the conditions of preparation, mixtures of the various types of sulfides are sometimes formed 35 having, for example, arbitrary formulae such as Ni<sub>3</sub>S<sub>2</sub>, which is believed to be a mixture of Ni<sub>2</sub>S and NiS. Other mixtures are known to exist, such as Fe<sub>3</sub>S<sub>4</sub>. It is essential that these sulfides be dispersed in the lubricating medium in gel 40 form, the inorganic skeleton of which is substantially the same as that of an aerogel. While the sulfides may be prepared by the previously known aerogel process, it is possible to prepare the present compositions without resorting to 45 the expensive drying operations usually involved in the preparation of an aerogel. However, if the exact steps involved in the preparation of a dry aerogel are to be avoided, they should be such as to permit the formation of a gel skeleton 50 structure similar to that of an aerogel.

The lubricating oils useful as the fluid lubricant in the present compositions comprise hydrocarbon oils of either natural or synthetic origin. Preferably, these oils have a viscosity between 55 about 60 SSU and about 3,000 SSU at 100° F.

and still more preferably between 300 SSU and 1,000 SSU at 100° F. These lubricating oils should have a medium or high viscosity index, preferably between 25 and 150. While the usual source for such oils is from petroleum crudes, other hydrocarbon oils may be used as well. These include especially polymerized olefins and particularly polymers of normal aliphatic olefins having from 6 to 12 carbon atoms and copolymers thereof with olefins having from 2 to 6 carbon atoms. Polymers having high viscosity indices and low pour points derived from such sources may be prepared by either catalytic or non-catalytic means. They may, for example, be prepared by heating the olefins at temperatures between 600° and 900° F. in the absence of catalysts or in the presence of such catalysts as lead tetraacetate at lower temperatures such as 400° F.-600° F. The clay-type catalysts of either natural or synthetic origin such as silica-alumina catalysts may be used as well. The advantages of employing lubricants comprising polymeric olefins are principally that of quality control as compared with the variable nature of lubricants obtained from natural sources which vary from one oil field to another and even from one well to another within a given field.

The lubricants are preferably at least moderately refined but, except when used as dielectric compositions, need not be highly refined; however, highly refined lubricating oils are equally suitable. While the principal object of the present invention has been stated to be the production of grease-like lubricants, another type of composition contemplated is that of thixotropic gels especially useful as cutting fluids or, more particularly, for well-drilling operations. In the latter instance especially, lower molecular weight hydrocarbon fluids are especially desirable and particularly those in the kerosene stove oil or gas oil boiling ranges. Compositions containing oils of such low boiling properties have been found to exhibit desirable thixotropic properties, especially useful in the operation of well-drilling mechanisms.

The sulfides to be used in the present compositions are metallic sulfides having a water solubility less than 0.0005 gram per 100 cc. of water at 20° C. Of particular importance is the group of sulfides of metals of the "hydrogen sulfide group," namely those metals precipitated by hydrogen sulfide as sulfides from their solutions in 0.3N acid. The latter group includes mercury, lead, copper, bismuth, cadmium, arsenic, antimony and tin. In addition to this group, other suitable sulfides are those of iron, nickel and cobalt.

The essential characteristic of an aerogel structure and of structures suitably similar thereto is that of maximum expansion so as to permit ready dispersal in a liquid medium and the maintenance of a permanent dispersion thereby. An aerogel is preferably formed by replacing water in a hydrogel with a low boiling water-miscible solvent such as ethyl alcohol or acetone, heating the resulting organo gel under pressure to a temperature above the critical temperature of the solvent, and at this point flashing off the solvent, leaving a highly expanded dry gel structure usually known as an aerogel. This structure is opposed to the structures ordinarily employed for catalysts which are termed "xerogels." In the latter instance, the gels are generally heated at extremely high temperatures with no effort being taken to maintain an expanded structure; hence, these products are hard, shrunken structures ordinarily totally unsuitable for use as grease-forming agents even

though they may be comminuted to the smallest size attainable by mechanical means.

Alternative means of preparing suitable gels for use in the present compositions comprises forming a hydrogel of the sulfide, displacing water with a water-miscible solvent such as alcohol or acetone and then replacing the solvent with a lubricating oil. Alternatively, the gels may be originally prepared under anhydrous conditions such as by reaction of an organic acid salt of the desired metal with hydrogen sulfide in a non-aqueous medium, such as ethyl alcohol. The anhydrous gel so formed is then transferred to oil and the surrounding low boiling medium removed. A specific instance of this process is given hereinafter, wherein copper acetate was dissolved in alcohol and then reacted with hydrogen sulfide.

Due to their oleophilic character, the "hydrogen sulfide group" metal sulfides may be formed into greases by especially economical methods. It has been discovered that the hydrogels of copper sulfide (for example) tend to shed water upon the addition of oil; hence, a copper sulfide hydrogel may be directly transferred to oil and water removed therefrom by simple decantation or distillation under reduced pressure. The oil and hydrogel are preferably milled to produce a finely dispersed mixture prior to water removal.

Still another process for use in the preparation of the present compositions comprises the transfer of a hydrogel into oil under so-called "direct transfer" conditions by use of suitable surface-active agents. The presence of surface-active agents such as high molecular weight amines and their derivatives enables the production of the present compositions by simple incorporation of the sulfide hydrogel in oil followed by milling to produce a fine dispersion of the hydrogel in the oil and subsequent removal of the water, preferably by distillation under reduced pressure. Suitable surface-active agents for use in this latter process include cationic surface-active materials such as high molecular weight amines, amine salts and quaternary ammonium compounds. While the cationic surface-active agents are especially preferred, non-ionic or anionic agents may also be used. Typical species of these agents include heptadecylamine, heptadecylimidazoline, amido amines of diethylenetriamine and oleic acid, soaps such as ammonium-12-hydroxystearate or lead oleate, soaps of hydroxy amines such as diethanolamine oleate, and glycerine monostearate.

The compositions of the present invention may vary within wide limits of one component to another, dependent upon the specific use for which the compositions are to be employed. Preferably, however, the compositions comprise a major amount of the hydrocarbon lubricating oil, and a minor amount of the colloidally dispersed sulfide. More specifically, effective compositions comprise 55-98% by weight, based on the total composition, of a mineral lubricating oil and 2-45% by weight of the sulfide. Generally, these compositions will contain from 65 to 85% by weight of the oil and 15 to 35% by weight of the sulfide. When the surface-active agents are present, they are ordinarily employed in amounts between about 2% and 40% by weight of the sulfide or from 1 to 5% based on the total grease.

Other ingredients may be present in these compositions including other grease-forming agents such as other inorganic gelling agents or high molecular weight soaps. The former include gels having structures similar to an aerogel and also similar (in their gelling action) to the subject

sulfides. These include aerogel-like structures of silica, alumina, magnesia, lime, aluminum silicates, alkaline earth metal oxides and hydroxides and similar inorganic gelling agents of either natural or synthetic origin. The natural materials include the swelling-type clays such as Wyoming bentonite and hectorite, which have been converted to oleophilic gelling agents by ion-exchange with oleophilic cationic surface active agents as represented by quaternary ammonium bases such as dimethyldiethylammonium chloride. When these auxiliary gelling agents are present, they may be used in an amount supplementary to the colloidal sulfide and may be included in the maximum ratio of said sulfide of between 5% and 45% by weight of the total composition. A typical grease of this character includes a composition comprising 70% mineral lubricating oil, 10% silica aerogel and 20% copper sulfide aerogel. The term "aerogel" is used throughout the specification to denote the type of porous gel structure desired rather than the specific method by which the gel was prepared.

Typical and illustrative but not limitative preparations of the sulfide greases are as follows:

#### EXAMPLE I

Fifty-six parts by weight of ferrous sulfate heptahydrate was dissolved in 100 parts of water made slightly acidic with sulfuric acid to repress hydrolysis. To this solution a solution of 38.7 parts of hydrogen sulfide dissolved in 434 parts of concentrated aqueous ammonia was added slowly with stirring. The temperature was maintained at about 0° C. After addition of the sulfide solution was completed, the reaction mixture was stirred for an additional 15 minutes. The ferrous sulfide gel was then filtered, washed with 750 parts of water saturated with hydrogen sulfide and finally with 1,000 parts of methyl alcohol. The alcogel so prepared was intimately mixed with a refined mineral lubricating oil having a viscosity of 300 SSU at 100° F. The mixture was heated to 74° C. and then at a temperature of 50° C. under vacuum for 14 hours to remove the last traces of alcohol. The resulting mixture was then milled to a grease-like structure and had a concentration of 21% by weight ferrous sulfide based on the total grease.

#### EXAMPLE II

408 parts by weight of nickel nitrate hexahydrate was dissolved in 700 parts of water. To this solution a solution of 190 parts of hydrogen sulfide dissolved in 2,140 parts concentrated aqueous ammonia were added slowly with stirring. The resulting gel of nickel sulfide so prepared was dehydrated with methanol and dispersed in lubricating oil as described in Example I. The resulting grease contained 35.7% by weight nickel sulfide.

#### EXAMPLE III

Copper sulfate pentahydrate was dissolved in water to form a concentrated solution. To this was added just enough concentrated aqueous ammonia to produce a copper-ammonia complex. Hydrogen sulfide was then bubbled into the solution. The resulting gelatinous precipitate was thoroughly washed with distilled water. Oil was mixed with the washed precipitate and the mixture was warmed. As heating progressed, it was possible to decant off most of the water. Progressive addition of oil followed by milling and dehydration under vacuum produced a grease gel containing 23% copper sulfide in oil.

#### EXAMPLE IV

Thirty-five parts by weight of copper acetate monohydrate was dissolved in 3,500 parts by weight of ethanol. Hydrogen sulfide was bubbled through this solution to obtain a gelatinous precipitate of substantially anhydrous copper sulfide alcogel. A mineral lubricating oil was added to alcogel so prepared and most of the alcohol was then decanted. The remainder of the alcohol was then removed by heating on a sand bath. The resulting mixture was milled to produce a grease containing 27.3% cupric sulfide.

#### EXAMPLE V

In order to determine the extreme pressure properties of the compositions prepared as described above, each of the greases was diluted with mineral lubricating oil to a gel concentration of 1.5%. These were tested in three-inch spur gears at 3,000 r. p. m. and 45° C., increasing the loading until scoring of the surfaces occurred. The extreme pressure loads of the greases were as follows:

|    | Composition                                            | Extreme Pressure Load, Lbs. |
|----|--------------------------------------------------------|-----------------------------|
| 30 | Mineral lubricating oil                                | 5                           |
|    | Nickel sulfide grease (Example II)                     | 45                          |
|    | Ferrous sulfide grease (Example I)                     | 45                          |
|    | Copper sulfide grease (Example IV)                     | 30                          |
|    | Best commercial extreme pressure additive <sup>1</sup> | 50                          |

<sup>1</sup> Mixture of benzyl disulfide, chlorodibenzyl disulfide and chlorinated paraffin wax.

This application is a continuation-in-part of copending application, Serial No. 782,694, filed October 28, 1947, which has matured into U. S. Patent 2,554,222, issued May 22, 1951.

We claim as our invention:

1. A lubricating grease composition comprising a major proportion of a hydrocarbon lubricating oil and as the principal gelling agent therefor a minor amount sufficient to form a grease structure of a colloidally dispersed copper sulfide, said gel being one which has its normal water content replaced by said oil.

2. A lubricating grease composition comprising a major proportion of a hydrocarbon lubricating oil and as the principal gelling agent therefor a minor amount sufficient to form a grease structure of a colloidally dispersed nickel sulfide, said gel being one which has its normal water content replaced by said oil.

3. A lubricating grease composition comprising a major proportion of a hydrocarbon lubricating oil and as the principal gelling agent therefor a minor amount sufficient to form a grease structure of a colloidally dispersed iron sulfide, said gel being one which has its normal water content replaced by said oil.

4. A lubricating grease composition comprising 55-98% by weight of a mineral lubricating oil and 2-45% by weight of a colloidally dispersed metallic sulfide having a water solubility less than 0.0005 gram per 100 cc. of water at 20° C., said gel being one which has its normal water content replaced by said oil.

5. A lubricating grease composition comprising 65-85% by weight of a mineral lubricating oil and 15-35% by weight of a colloidally dispersed metallic grease-forming sulfide having a water solubility less than 0.0005 gram per 100 cc. of water at 20° C., said sulfide having a colloidal

gel structure substantially the same as that of the gel as originally formed.

6. A lubricating grease composition comprising a major proportion of a hydrocarbon lubricating oil and as a gelling agent therefor a minor amount sufficient to form a grease structure of a 5 colloidal dispersed metallic sulfide having a water solubility less than 0.0005 gram per 100 cc. of water at 20° C., said sulfide having a colloidal gel structure substantially the same as that of 10 the gel as originally formed.

7. A lubricating grease composition comprising a major proportion of a hydrocarbon lubricating oil and as a gelling agent therefor a minor amount sufficient to form a grease structure of a 15 colloidal dispersed metallic sulfide having a water solubility less than 0.0005 gram per 100 cc. of water at 20° C., said sulfide having a colloidal

gel structure wherein the gel particles have dimensions between 0.001 and 0.1 micron each, the metallic radical of said sulfide being a metal of the group of metals precipitated by hydrogen sulfide as sulfides from their solutions in 0.3N acid, said gel being one which has its normal water content replaced by said oil.

FRED H. STROSS.

STANLEY T. ABRAMS.

References Cited in the file of this patent

UNITED STATES PATENTS

| Number    | Name     | Date          |
|-----------|----------|---------------|
| 2,260,625 | Kistler  | Oct. 28, 1941 |
| 2,554,222 | Stross   | May 22, 1951  |
| 2,573,650 | Peterson | Oct. 30, 1951 |
| 2,584,085 | Stross   | Jan. 29, 1952 |